

April 7, 1925.

1,532,819

J. H. HASTE

PROCESS FOR PREPARING PHOTOGRAPHIC FILMS

Filed April 14, 1924



INVENTOR,  
James H. Haste,  
BY *R. L. Stinchfield*

ATTORNEY

Patented Apr. 7, 1925.

1,532,819

# UNITED STATES PATENT OFFICE.

JAMES H. HASTE, OF ROCHESTER, NEW YORK, ASSIGNOR TO EASTMAN KODAK COMPANY, OF ROCHESTER, NEW YORK, A CORPORATION OF NEW YORK.

## PROCESS FOR PREPARING PHOTOGRAPHIC FILMS.

Application filed April 14, 1924. Serial No. 706,378.

*To all whom it may concern:*

Be it known that I, JAMES H. HASTE, a citizen of the United States of America, residing at Rochester, in the county of Monroe and State of New York, have invented certain new and useful Improvements in Processes for Preparing Photographic Films, of which the following is a full, clear, and exact specification.

10 This invention relates to processes for preparing photographic films and is applicable to (but not limited to) the preparation of films of the type disclosed in my prior application, No. 591,862, filed Oct. 2, 1922 for composite film, of which the present application is a continuation in part.

One object of the invention is to provide a process for the rapid and economical production of a composite photographic film 20 in which the several layers are made to adhere with especial tenacity and without destroying said layers. Other objects will hereinafter appear.

In the accompanying drawing,—

25 Fig. 1 is a fragmentary cross section, upon an exaggerated scale, of one form of film which may be produced by my process;

30 Fig. 2 is a diagrammatic elevation upon an exaggerated scale of one form of apparatus in which the steps of my process may be conveniently carried out.

In the manufacture of photographic films in which the gelatino-silver halid emulsion layer is carried upon a laminated base or support, the layers of which comprise cellulose materials such as cellulose nitrate and cellulose acetate, it is essential for the best results to have all the layers adhere with reliable firmness so that they will not become separated when subjected to the action of photographic liquids, when drying, or when subjected to the heat of projection apparatus. This is especially true where such films are employed in the motion picture art.

45 But this adhesion ought not to be obtained at the expense of uniformity in the product, that is, the steps which promote the bonding of the layers ought not to impair or wash away any of the layers themselves. This is especially important where the sensitive photographic coating is not applied directly to the base, but is coated onto a gelatinous bonding substratum previously formed on the base. For example, the problem is particularly difficult when a substratum is

formed on laminated film supports in which the cellulosic layer on the face nearest the light sensitive coating is very thin, like an outer layer, for instance, of the film base in my hereinabove cited prior application. 60 Precautions must then be taken in applying the substratum forming liquid to prevent washing away the thin layer. On the other hand, the substratum forming liquid must sufficiently affect the layer to obtain the necessary bond or adhesion with it. 65

I have found that the problem can be reliably solved by correlating the formation of the thin cellulosic layer and the formation of the substratum. The cellulosic coating is formed by applying a dope or varnish to the main layer of the base. From this coating part of the volatile liquid is evaporated to stabilize it; and then there is applied to it a gelatinous substratum-forming composition insufficient to remove the partially stabilized coating, but including sufficient volatile solvent to promote adhesion between it and the coating. Any residue of volatile liquid in the cellulosic coating and the volatile 70 liquid in the substratum are finally evaporated simultaneously to produce an especially strong interunion.

The principle of such procedure is of general applicability wherever a gelatino-silver 35 halid emulsion layer has to be united by means of a substratum layer to a cellulosic varnished or thinly coated face of a support. Moreover this principle applies whether the cellulose layers, coatings, and varnishes of 80 the base or support be composed of such compounds as cellulose nitrate, cellulose acetate, cellulose ether, or various mixtures of them with or without softeners. Since, however, the principle is especially valuable in 85 preparing the film described in my hereinabove cited prior application, I shall describe the application of it to the manufacture of such film; but it will be understood that this is done by way of illustration, and 90 that the described steps are equally applicable to the preparation of other films, the manufacture of which presents the same 95 broad problem.

100 Referring to the accompanying drawing, 105 a sheet or band 1 of cellulose acetate composition (such for instance as that disclosed in U. S. Patent No. 1,342,601, Seel, June 8, 1920) which is to form the main layer of the film base is passed over any suitable guid- 110

ing and propelling means, such as the roller 10, which carries it over any suitable coating means, such as roller 11, partially immersed in a bath 12 of nitrocellulose solution or varnish, the nitrocellulose being of the known coatable types used in films, lacquers, and photography.

This varnish may, for instance, be similar to the one disclosed in my hereinabove cited prior application, and, therefore, contain 100 parts of nitrocellulose dissolved in 30 to 100 parts of fusel oil or butyl alcohol and 400 to 5000 parts of a mixture of acetone and methyl alcohol in varying relative proportions, say equal parts by weight. When the reduction of inflammability is of importance, as in the preferred film described in my hereinabove cited application, there is also added to this dope or varnish 10 to 50 parts of triphenyl phosphate. As will be understood by those skilled in the art, the above varnish can be thinned out even further to obtain greater flowability by the addition of still more acetone and methyl alcohol, or even by the addition of some diluent like ethyl alcohol. It is flowable so as to be especially convenient for application by means of a coating wheel, as indicated at 11. Of course, any other equivalent known coating expedients can be used in place of a wheel, such as slotted troughs, belts, coating brushes, spraying apparatus, etc.

The layer 1 carrying the coating of nitrocellulose 2 next moves toward guiding or propelling means 13, indicated here as a wheel, like wheel 10, having a smooth supporting periphery. During its passage from wheel 10 to wheel 13 the nitrocellulose coating 2 becomes hardened, so that it can pass without harm in direct contact with the periphery of the wheel. This coating 2 is one of the sealing layers described in my hereinabove cited prior application and could be formed after, as well as before, the other coating steps, because it plays no direct part in the solution of the hereinabove described problem. In fact a usable unsealed film can be made by omitting it and merely following the hereinafter described procedure. The hardening of the coating during its passage between the wheels 10 and 13 may, of course, be hastened by the application of heat, currents of drying gas, or other well known expedients, as will be understood by those skilled in the art without further description.

When the layer 1 bearing the coating 2 passes around the wheel 13, its uncoated face is outward and held evenly so that it is adapted to receive a uniform coating 3 by any suitable means, here illustrated as a roller 14 turning in bath 15. The latter may have the same composition as that of bath 12 described hereinabove. Layer 1

carrying the hardened layer 2 and the still uncured or somewhat plastic layer 3 then passes to suitable guiding or propelling means 16, which may likewise be a roll having a smooth supporting periphery, cooperating with coating roll 17. The above mentioned rolls may of course be power driven, and the speeds of the rolls may be individually adjustable as well as the spacing of the coating rolls from the film, known coating machine practice being followed in these respects.

As the coated film base or support passes toward roll 16, the coating 3 starts to set or harden because of the evaporation of the volatile liquids from it. This may be assisted, if desired, by the application of heat or currents of drying gas. The evaporation is not, however, carried through to the point where the coating 3 becomes fully hardened. It should still be in a somewhat uncured or partially undried state when it reaches roll 16. This enables it to receive the substratum-forming liquid without being washed away by the latter, and still be in a state to promote adhesion. Its partially set condition, in which it thus resists washing away and yet promotes adhesion, is conveniently termed a partially stabilized state. While adhesion can be effected to a degree that is sometimes useful when curing has taken place, nevertheless, the adhesion is stronger and the process is faster when the substratum is applied to a coating which is only partially stabilized.

As the film base or sheet passes below the roll 16, a substratum forming liquid is applied to the partially stabilized layer 3 by any suitable means, such as a coating roll 17, turning in bath 18.

The substratum-forming composition is preferably of a kind described in U. S. Patent No. 550,288, Penniman, Nov. 26, 1895. It may, for example, consist of gelatine in a liquid containing a solvent of celluloid, such as acetic ether or other well known equivalent volatile nitrocellulose commercial solvents. The gelatinous liquid is preferably kept dilute (say under five per cent of gelatine) so as to have an easy flowing capacity, the strength being a matter of routine adjustment by any one skilled in the art to meet slightly varying conditions. The thicker the solution employed, the faster the film band should pass over roll 17, and the slower the roll 17 should feed. The thicker layer 3 is, the thinner the gelatinous solution may be. Of course, if the layer 3, to which the substratum 4 is to adhere, be composed of a different cellulosic material from nitrocellulose, corresponding known volatile solvents of such material will be substituted in the substratum in place of the nitrocellulose solvents mentioned by Penniman.

By adjusting roll 17, the substratum-forming composition is applied in the right quantity to avoid the eating out or washing away of the partially stabilized coating 3. As the film band passes away from rolls 16 and 17, the volatile liquids remaining in layer 3, as well as the volatile liquids in the substratum 4 evaporate together. It has been found that this simultaneous evaporation, carried out under the described conditions, effects an especially durable bond between the strata without impairing the latter. The evaporation may, of course, be conducted by heating, or currents of drying gas, or other expedients well known in the art. At all points where volatile solvents are evaporated, the vapors may be conducted away and recovered in the ways known in the art. When the evaporation of volatile liquids from coating 3 and substratum 4 has reached such a point that the convolutions will not stick together or be impaired by intercontact, the sheet or film 1 may be rolled up for storage, or the gelatino-silver halid emulsion may optionally be applied immediately to substratum 4, as at coating 5 without coiling up the sheet. The coating with the emulsion follows customary known practice.

Of course the substratummed sheet is adapted to firmly adhere to other gelatinous coatings applied thereto instead of light-sensitive emulsions. Gelatine for the bichromate process and dyed gelatine, say for filters, are illustrative of photographic gelatinous layers which can be substituted.

Having thus described my invention, what I claim as new and desire to secure by Letters Patent is:

1. In the process of making a film having a gelatinous layer attached by a substratum to a laminated support which has a coating of cellulosic material on a main layer, the steps of forming said coating by applying to said main layer a relatively thin coating of cellulosic material dissolved in a volatile liquid which contains a solvent of said main layer to promote adhesion between said coating and layer, partially stabilizing said coating by evaporating a portion of said liquid therefrom, applying over said partially stabilized coating a gelatinous substratum-forming composition, insufficient to remove said coating, said composition including a volatile liquid containing a solvent of said coating to promote adhesion between it and said substratum, and simultaneously evaporating said volatile liquids from said superposed coating and substratum.

2. In the process of making a film having a photographic gelatinous layer attached by

a substratum to a coating of nitrocellulose on a main cellulosic layer, the steps of applying to said main layer a relatively thin coating of nitrocellulose dissolved in a liquid which contains a solvent of said main layer to promote adhesion between said coating and layer, partially stabilizing said coating by evaporating a portion of said liquid therefrom, applying over said partially stabilized coating a gelatinous substratum-forming composition insufficient to remove said coating, said composition including a volatile liquid containing a nitrocellulose solvent to promote adhesion between said coating and said substratum, and simultaneously evaporating said volatile liquids from said superposed coating and substratum.

3. In the process of making a film having a light sensitive gelatino-silver-halid layer attached by a substratum to a nitrocellulose coating on a main acetone-soluble cellulose acetate layer, the steps of applying to said main layer a relatively thin coating of nitrocellulose varnish containing acetone to promote adhesion between said coating and main layer, partially drying said coating, applying over said partially dried coating a gelatinous substratum-forming liquid composition insufficient to remove said coating but containing a volatile nitrocellulose solvent to promote adhesion between said coating and said substratum, and drying together said superposed coating and substratum.

4. In the process of making a film having a light sensitive gelatino-silver-halid emulsion layer attached by a substratum to a coating of cellulose-ester on a main cellulosic layer, the steps of applying to said main layer a relatively thin coating of cellulose ester dissolved in a volatile liquid which contains a solvent of said main layer to promote adhesion between said coating and layer, partially stabilizing said coating by partially evaporating said liquid, applying over said partially stabilized coating a gelatinous substratum-forming composition insufficient to remove said coating, said composition including a volatile liquid containing a solvent of said coating to promote adhesion between it and said substratum, simultaneously evaporating said volatile liquids from said superposed coating and substratum and coating a light sensitive gelatino-silver-halid emulsion over said substratum.

Signed at Rochester, New York this 9th day of April, 1924.

JAMES H. HASTE.